

Feb. 7, 1961

R. GUMBINER

2,970,931

STENCIL SHEET HAVING TRANSFERABLE BACK COATING

Filed March 25, 1957



INVENTOR.  
ROBERT GUMBINER

BY *Attalaund, Baker,  
Kurt & Saffer*  
ATTORNEYS

# United States Patent Office

2,970,931

Patented Feb. 7, 1961

1

2,970,931

## STENCIL SHEET HAVING TRANSFERABLE BACK COATING

Robert Gumbinner, Tarrytown, N.Y., assignor to Poly-chrome Corporation, Yonkers, N.Y., a corporation of New York

Filed Mar. 25, 1957, Ser. No. 648,250

3 Claims. (Cl. 117—35.5)

This invention relates to a stencil assembly which includes a novel stencil sheet adapted to produce a carbon impression simultaneously with the cutting of the stencil.

A stencil sheet generally is formed of a base tissue made of a long fiber such as manila hemp. This base tissue is coated by various methods such as roller, fountain and spray coating with a composition that is displaceable when acted upon by a typewriter, stylus or the like, so as to form an opening through which duplicating ink may flow.

It is known to assemble such stencil sheets by adhesively securing one marginal edge thereof to a carbon cushion sheet and to a backing sheet. The purpose of the carbon cushion sheet is to provide a contrast in visibility when typing the stencil and also to produce an impression on a backing sheet which can then be used as a proof copy or for other desired purposes. For example, the stencil and carbon backing sheet are sometimes attached to an invoice form so that, when the stencil is typed, a copy is obtained on the invoice and the stencil can then be used in a hand stamp or otherwise to provide copies on packing containers.

Prior to the present invention, it was not possible to successfully provide a stencil assembly of this type which would eliminate the necessity for a separate carbon sheet. However, there is now provided on the back of the stencil sheet itself a dark, impression-transmitting coating which in a far more simple and economical fashion performs the function of the separate carbon sheet heretofore necessary.

Previous attempts to coat the backing sheet of a stencil assembly with a carbonized material have not proven successful, because the oils in the stencil coating tended to soften the carbon on the backing material. Thus, while contrast would be obtained during the typing of the stencil, it would not be possible by such methods to obtain the type of proof copy referred to above.

Accordingly, it is an object of the present invention to provide a stencil assembly which includes a stencil sheet having a dark, image-transmitting coating on one surface thereof which will perform the function of the extra carbon sheet heretofore necessary.

Another object is to provide a stencil assembly which includes an image-transmitting stencil sheet and a backing sheet upon which a proof copy may be formed simultaneously with the cutting of the stencil.

These and other objects of my invention will become apparent from the following description when taken in connection with the drawing, in which the single figure is a perspective view showing the construction of the stencil as it would appear with the stencil sheet in the partially removed position.

Essentially the present invention is directed to a stencil sheet comprising a base tissue having a pastel-colored stencilizable coating on the surface thereof which is to receive the impression from the typewriter, stylus or the like. On the opposite, or back surface thereof, a

2

carbon, impression-transmitting coating is provided. Although this coating typically, but not necessarily, includes a carbon type pigment, for the sake of simplicity it will hereinafter be referred to as the "carbon" coating.

This stencil sheet is readily fastened to a suitable impression-receiving backing material by providing, on one marginal edge thereof, a coating of a pressure sensitive adhesive which allows the stencil to be removably

10 secured to the backing.

Thus, when making stencils in accordance with the stencil sheet and assembly herein disclosed, the carbon coating on the back of the stencil sheet provides sharp contrast with the pastel coated surface normally visible to the stencil cutter and at the same time allows for the production of carbon proof copies on the impression receiving backing sheet.

Referring now to the drawing, it is seen that stencil sheet 10 may be removably secured to backing sheet 11 by means of the pressure sensitive adhesive strip 12, so that after the stencil is cut, the stencil sheet is readily removed from the backing. The backing sheet also is readily detachable by means of perforations 16. It is also seen from the figure that there is produced on the 25 backing sheet a carbon impression 18 of the stencil which was cut.

The pastel coating which is applied to the normally visible or outside surface 14 of the stencil sheet will typically be an oil-fatty acid-nitrocellulose mixture having 30 included therewith the desired light colored pigment in suitable proportions. An example of a suitable composition for the pastel-colored coating is as follows:

| Material:      | Percentage by weight |
|----------------|----------------------|
| Nitrocellulose | 12                   |
| 35 Oleic acid  | 70                   |
| Castor oil     | 12                   |
| Pigment        | 6                    |

In addition to the above, of course various stabilizers 40 and plasticizers such as tricresyl phosphate, phenol, chlorinated naphthalene may be used.

The pigment which may be used to impart the desired pastel color would be lead chromate, titanium dioxide, Hansa yellow or other lighter shades.

45 In applying this coating, the pigment is first ground thoroughly on a three roll mill in a portion of the oil. The nitrocellulose is dissolved in a mixture of active and latent solvents such as ether, ethyl alcohol, butyl acetate, methyl acetate, acetone, ethylene glycol, mono-50 ethyl ethers, ethyl ethers, ethyl lactate, isopropyl alcohol. Other solvents such as are typically used in lacquer formulations may also be used.

In addition to the above, a hydrocarbon diluent may be used in quantities sufficiently limited not to upset the 55 gel formation necessary for the production of a good stencil coating.

The pastel coating is preferably applied to the stencil sheet before the carbon coating. In order to make sure that the pastel coating is applied only to one side of the 60 fiber sheet, it is necessary to set this coating rapidly after the application of the coating solution. Since the coating may be applied at various temperatures, there are many solvents which may be selected which are sufficiently volatile to provide the necessary rapid setting. For example, using temperatures of the order of 150° F., ethyl 65 alcohol and ether would be suitable solvents while at higher temperatures up to about 250° F. higher boiling solvents may be selected to obtain the same desired results.

The opposite or back side of the stencil sheet 15, which is not normally visible to the stencil cutter and which is in direct contact with the backing sheet, is pro-

vided with a dark impression-transmitting coating which would typically have the following composition.

| Material:      | Percentage by weight |
|----------------|----------------------|
| Nitrocellulose | 14                   |
| Oleic acid     | 61                   |
| Castor oil     | 15                   |
| Dark pigment   | 10                   |

Note that in the carbon coating, the ratio of nitrocellulose to the fatty acid and oil is higher than in the pastel coating. This is necessary to make a relatively hard coating which will give a sharp impression on the copy paper and will not result in a broad splash or blurred carbon image of the stencil.

In applying this carbon coating to the stencil sheet, the same solvents as used with the pastel coatings may be used, except that the percentage of the latent solvents should be higher in order that this coat does not attack or interact with the previously applied pastel coating.

The dark pigments which are used in the impression-transmitting coating are commonly black pigments such as carbon black, lamp black or Peerless black. In addition to the above, blue pigments such as iron blue can be used and, if desired, a green pigment such as a mixture of iron blue and a yellow pigment may also be used to give a satisfactory color and sufficient density for good visibility.

It is, of course, necessary to limit the pigments in both coatings to those which will not bleed in the oils used to plasticize the nitrocellulose.

In addition to the pigments mentioned above, there may also be used tungstated Victoria blue or a non-bleeding red pigment such as certain Lithol reds which are well known to the art.

Both the pastel and dark colored pigments should be applied to the stencil sheet so that a suitable weight of coating is applied on each side thereof. Each gram of base tissue will have on the outside surface thereof about 2.7 to 5.0 grams of the pastel coating composition and between about .08 to 1.6 grams of the carbon coating composition. These quantities are typically applied to a stencil sheet eight and a half by sixteen and a half inches which will commonly have a weight of the order of one gram.

As previously mentioned, it is important that the ratio of oil (including fatty acid) to nitrocellulose should be higher in the pastel coating. Thus in this coating, the oil to nitrocellulose ratio will be in the range of about 6.5:1 to 9:1. The carbon coating will have a ratio of oil to nitrocellulose in the range of about 4:1 to 7:1.

In addition to the above, it is of course apparent to one skilled in the art that the oil to nitrocellulose ratio may be dependent to some extent on the viscosity of the coating composition. It is also apparent that there are a wide variety of oil plasticizers and grades of nitrocellu-

lose which can vary the specific proportions referred to in the above examples.

By coating the stencil sheet as indicated above, there is provided a single sheet which eliminates the necessity and therefore the cost of a separate carbon sheet. This advantage not only reduces manufacturing costs, but provides for simplicity in handling because there is no need to keep a separate carbon sheet in alignment with the stencil and the backing sheet.

Although preferred forms of this invention have been here disclosed, it will now be apparent to those skilled in the art that many modifications and variations may be made, and it is preferred therefore to be limited, not by the specific disclosure herein, but only by the appended claims.

What is claimed is:

1. A stencil sheet comprising a base tissue, a pastel-colored stencilizable coating on one surface of said base tissue, said coating having an oil to nitrocellulose ratio in the range of about 6.5:1 to 9:1, and on the opposite surface of the base tissue, a dark, impression-transmitting coating having an oil to nitrocellulose ratio in the range of about 4:1 to 7:1.

2. The stencil sheet of claim 1 in which the pastel-colored stencilizable coating is present in an amount of from about 2.7 to 5.0 grams per gram of base tissue and the dark, impression-transmitting coating is present in an amount between about .08 to 1.6 grams per gram of base tissue.

3. A stencil sheet comprising a base tissue, a pastel-colored stencilizable coating on one surface of said base tissue, said coating having an oil to nitrocellulose ratio in the range of about 6.5:1 to 9:1, said coating further being present in amounts of from about 2.7 to 5.0 grams per gram of base tissue and, on the opposite surface of the said base tissue, a dark, impression-transmitting coating having an oil to nitrocellulose ratio in the range of about 4:1 to 7:1, said coating further being present in an amount of between about .08 to 1.6 grams per gram of base tissue.

References Cited in the file of this patent

UNITED STATES PATENTS

|    |           |          |               |
|----|-----------|----------|---------------|
| 45 | 1,617,386 | Fuerth   | Feb. 15, 1925 |
|    | 1,645,593 | Geiger   | Oct. 18, 1927 |
|    | 1,664,777 | Horii    | Apr. 3, 1928  |
|    | 1,828,766 | De Waele | Oct. 27, 1931 |
| 50 | 1,937,751 | Elliott  | Dec. 5, 1933  |
|    | 2,313,810 | Dalton   | Mar. 16, 1943 |
|    | 2,335,992 | Biskind  | Dec. 7, 1943  |

FOREIGN PATENTS

|    |         |               |               |
|----|---------|---------------|---------------|
| 55 | 392,220 | Great Britain | May 15, 1933  |
|    | 424,495 | Great Britain | Feb. 15, 1935 |